

Patented Nov. 26, 1929

1,736,934

## UNITED STATES PATENT OFFICE

PAUL I. MURRILL, OF PLAINFIELD, NEW JERSEY, ASSIGNOR TO R. T. VANDERBILT COMPANY, INCORPORATED, OF NEW YORK, N. Y., A CORPORATION OF NEW YORK

## PREPARATION OF PICKLING BATHS

No Drawing.

Application filed November 22, 1928. Serial No. 321,270.

This invention relates to the preparation of a pickling bath especially adapted for the cleaning or pickling of iron or steel to remove scale therefrom, although the bath may be applied more generally to the cleaning or picking of metals, such as iron or steel, for the removal of oxides or scale therefrom.

The pickling or cleaning of iron or steel is commonly effected by means of acid pickling or cleaning baths which remove scale or oxide from the metal. The pickling baths commonly employed are acid baths which often attack the metal as well as the scale. This action on the metal is undesirable and objectionable, involving not only excessive consumption of the acids, but also corrosion or solution of the metal and tending to give a rough or pitted surface.

According to this invention an acid pickling or cleaning bath is made by adding to the acid, a mercaptothiazole and particularly a mercaptobenzothiazole in the form of a salt. In preparing the pickling or cleaning bath, mercaptothiazoles, which are insoluble in water and sparingly or slowly soluble in dilute acids, and not wetted by water or dilute acids, but soluble in alkaline solutions, such as caustic soda, are dissolved in such an alkaline solution and added to the acid of the bath in this form. The acid may, and generally does set free the mercaptothiazole from the solution, but in a form such that it may more readily be dissolved in the acid of the bath than if added directly to the bath in the form of crystals or powder. The addition of a small amount of a suitable mercaptothiazole in the form of a salt, such as an alkali metal salt, prevents, retards or inhibits the attack of the acid of the bath on the metal without interfering in any substantial way with the removal of the scale or oxide by the acid bath.

The acid pickling baths with which the mercaptothiazoles are used, may be acid baths, such as are commonly employed for pickling or cleaning iron and steel and contain, for example, about ten per cent of sulfuric acid. Such baths are gradually impoverished by the action of the acid in removing the scale or rust and their content of ferrous sulfate increases until the bath be-

comes too weak or it becomes too concentrated in ferrous sulfate for further use. Instead of using sulfuric acid baths, other baths may be used including acid sulfate baths.

Only a small amount of a mercaptothiazole is necessary to exert the desired inhibiting effect on the acid of the bath. In general, only a small fraction of one per cent is required. In the case of mercaptobenzothiazole, for example, about two to five pounds of the compound are sufficient for each ton of 60° sulfuric acid used in the pickling bath. The mercaptothiazole employed should be one which is stable and does not decompose to any objectionable extent in the acid bath, and in addition, should be one which forms a soluble salt in alkaline solution.

In dissolving the mercaptothiazole in alkali prior to adding it to the acid pickling bath, sufficient alkali should be employed to dissolve the compound, although an excess of alkali may be employed without harmful effect. In dissolving 2-mercaptobenzothiazole, for example, the solution may be prepared by dissolving 25 parts by weight of the compound in 75 parts by weight of 10% caustic soda. This will give a solution of approximately the following composition:

|                       | Per cent |
|-----------------------|----------|
| Mercaptobenzothiazole | 25.0     |
| Sodium hydroxide      | 7.5      |
| Water                 | 67.5     |

Other mercaptothiazoles may be employed in a similar way such as 2-mercato-4-methylbenzo-thiazole, 2-mercato-4,6-dimethylbenzo-thiazole or 2-mercato-5-phenylthiazole.

As it is customary to employ pickling baths at an elevated temperature, for example, around 150 to 180° F., the bath may be heated during the addition of the mercaptothiazole inhibitor without any additional expense. This, however, is not necessary as the inhibitor may be added to the bath at room temperature.

I claim:

The method of incorporating a mercaptobenzothiazole in an acid pickling or cleaning bath which comprises dissolving the mercap-

tobenzothiazole in caustic alkali to form a solution thereof in the form of the alkali metal salt and adding the resulting solution with stirring to the acid bath whereby the reaction of the acid of the bath with the alkali metal salt of the mercaptobenzothiazole sets free the mercaptobenzothiazole in a form which promotes its solution in the acid bath.

In testimony whereof I affix my signature

**PAUL I. MURRILL.**

**10**

**15**

**20**

**25**

**30**

**35**

**40**

**45**

**50**

**55**

**60**

**65**